

June 2, 1931.

J. F. WITT

1,807,947

PAVING METHOD

Filed Jan. 30, 1930 2 Sheets-Sheet 1



Fig. 1



Fig. 2



Fig. 3



Fig. 4

Inventor

J. F. Witt

By

Jack A. Schley  
attorney

June 2, 1931.

J. F. WITT

1,807,947

PAVING METHOD

Filed Jan. 30, 1930 2 Sheets-Sheet 2



Fig. 5



Fig. 6

Inventor  
J. F. Witt

By

Fig. 7

Jack A. Schley  
Attorney

## UNITED STATES PATENT OFFICE

JACKSON F. WITT, OF DALLAS, TEXAS

## PAVING METHOD

Application filed January 30, 1930. Serial No. 424,609.

This invention relates to new and useful improvements in paving methods.

One object of the invention is to secure a top or surface layer to a supporting course in a new and novel manner, whereby liquid asphalt may be effectively used and not only spread to a uniform thickness but so maintained even on crowned roads.

A further object of the invention is to so 10 interlock the liquid asphalt layer as to prevent creeping or disintegration of said layer.

Another object of the invention is to embed the liquid asphalt in depressions in the supporting course, whereby the paving is 15 tied together, the co-hesion enhanced and the wearing surface increased.

A construction designed to carry out the invention will be hereinafter described together with other features of the invention.

20 The invention will be more readily understood from a reading of the following specification and by reference to the accompanying drawings in which an example of the invention is shown, and wherein:

25 Figure 1 is a transverse sectional view of a supporting course ready for carrying out my improved method.

Figure 2 is a similar view showing the 30 priming coat applied.

Figure 3 shows the same after the puncturing or penetrating step.

Figure 4 is a transverse sectional view of a finished pavement.

35 Figure 5 is an enlarged sectional detail of its finished pavement.

Figure 6 is an isometrical view of a tool used in the method, and

40 Figure 7 is a transverse sectional view of a modified form of pavement.

In carrying out the method a supporting course A is first built up in the usual manner. This course may be of any soft or semi-soft material, such as soft limestone, 45 caliche, water-bound macadam, gravel or

shell foundation or any other material capable of being punctured or indented.

Where the course is of clay formation or materials which become glazed when rolled, it is necessary to scrape the surface sufficiently to leave a granular or saw-tooth top. This 50 may constitute the first step of the method or it may not be necessary as where soft limestone is used.

With the top surface of the course A prepared, a suitable hot liquid asphalt or asphaltic road oil is sprayed or spread over the said surface to form a prime coat or layer B.

This coat is comparatively thin, one-quarter 60 of an inch having been found satisfactory, but the invention is not to be limited to this measurement.

Immediately after the liquid asphalt is applied, there will be spread or cast over the 65 entire surface of said prime coat, either pea gravel, coarse sand or limestone screenings or the like in sufficient quantity to absorb the free liquid asphalt on the surface of the coat. The next step consists in rolling the 70 surface of the coat B with a suitable roller, whereby it is smoothed and the mineral aggregate is embedded therein.

The prime coat B is now ready for the 75 next step, which consists in puncturing or penetrating the coat and indenting the surface of the course A.

In Figure 6 I have shown a roller 10 having conical studs or points 11 on its cylindrical surface. These studs are preferably arranged in circumferential rows, and those of one row in staggered relation to those of the adjacent rows.

By giving the studs a suitable length or projection from the face of the roller they not 85 only penetrate the coat B, when rolled thereover, but indent the surface of the course A as is shown in Figure 3. Any other suitable tool may be used so long as the coat B is punctured. If the asphaltic oil should tend 90

to flow to the sides of pavement the sumps C will intercept it and thus prevent segregation of the base oils.

The next step consists in spraying or spreading over the prime coat B hot liquid asphalt or asphaltic road oil so as to accumulate to a thickness preferably greater than that of the prime coat and form a top layer or course D. Good results have been had with a layer one-half of an inch thick, but this measurement is optional.

When the course D is applied the asphaltic oil will flow down through the openings in the prime coat and fill the sumps C, thus forming inverted cones E depending from the top coarse. Asphalt having an affinity for itself, it is obvious that the cones will adhere to the prime coat, whereby the cohesion of the asphaltic oils will be set up. The coat B and course D will be interlocked thus holding them in place, and preventing disintegration.

After the course D is applied, pea gravel, limestone screenings or other fine mineral aggregate is spread over the surface. This is followed by rolling the surface until its free asphalt is absorbed, after which the pavement may be thrown open to traffic. The cones E extending down into the course A and being on comparatively close centers provide an adequate support and increase the wearing surface as well as preventing creeping or buckling of the pavement.

In some instances it may be desired to resurface or surface an old road or street, or to eliminate the prime coat. In such case the supporting course A as shown in Figures 7, is punctured by rolling with the roller 10 to form sumps C' therein. The top course D' is then applied direct to the supporting course and the cones E' formed by the asphalt flowing into said sumps. By this arrangement the top course is locked to the supporting course.

Depending upon the porosity and softness of the supporting course, the asphaltic oil will penetrate the walls of the sumps to a more or less extent, and thus establish by cohesion a bond therewith. By spreading mineral aggregate on the prime coat B a layer of mineral aggregate is thus embedded in the pavement and this tends to bind the coat B and course D together between the cones.

It is pointed out that when the mineral aggregate which has been spread upon the layer D is rolled it will be forced down into the cones thus stabilizing them and also reinforcing said cones against lateral strains.

What I claim, is:

1. The method of paving which consists in applying a prime coat of hot liquid asphalt to the top surface of a soft supporting course, then puncturing said coat and penetrating the underlying surface of the supporting course, and then applying a layer of hot liquid asphalt to the prime coat and flowing

the same through the punctures of said coat and into the penetrations in the supporting course to interlock the courses.

2. The method steps set forth in claim 1 with the step of spreading fine mineral aggregate on the prime coat, and rolling the same prior to puncturing. 70

3. The method steps set forth in claim 2 with the step of spreading fine mineral aggregate on the top layer and rolling the same until the free asphalt is absorbed. 75

In testimony whereof I affix my signature.

JACKSON F. WITT.

80

85

90

95

100

105

110

115

120

125

130